

# UNITED STATES PATENT OFFICE.

HENRY J. TILL, OF LOS ANGELES, CALIFORNIA.

## ADHESIVE COMPOUND FOR COLLAR-SUPPORTS.

983,955.

Specification of Letters Patent. Patented Feb. 14, 1911.

No Drawing.

Application filed February 8, 1910. Serial No. 542,769.

*To all whom it may concern:*

Be it known that I, HENRY J. TILL, a citizen of the United States, residing at Los Angeles, in the county of Los Angeles and State of California, have invented certain new and useful Improvements in Adhesive Compounds for Collar-Supports, of which the following is a specification.

This invention relates to compounds and 10 more particularly to an adhesive compound for application to collar stays or supports for retaining said supports in position on ladies' lace or fabric collars or on the collars of men's soft shirts.

15 The object of the invention is to provide a compound which is rendered soluble in water and adhesive under the application of moisture and heat so that the support may be positioned on a collar during the ironing operation and removed therefrom when the collar is laundered.

20 With the above object in view, the invention consists in a compound formed of the following ingredients in the proportions stated, to wit:—white glue 16 ounces, paraffin or other wax 8 ounces, glycerin 3 ounces, sufficient water being added to give the compound the desired consistency.

25 In carrying the invention into effect, the glue, paraffin and glycerin are placed in a suitable receptacle and heated, sufficient water being added thereto to render the adhesive of the proper consistency to be applied to the supports or stays with a brush or 30 gluing machine.

35 The paraffin or other wax is added for the purpose of making the collar support or other article to which the adhesive is ap-

plied moisture proof, thus guarding against the support becoming accidentally detached 40 from the collar when subjected to perspiration from the neck of the wearer. The glycerin is added to render the support pliable and thus prevent breakage or snapping of the support when twisting or turning the 45 head.

The adhesive is preferably applied to one side of the stay or support and fills the mesh of the fabric backing of the support so that the compound is held in suspension in the 50 fabric mesh and when cool presents a smooth hard surface.

Such a compound has been found, by experience, especially desirable as an adhesive for collar supports inasmuch as it is white 55 in color to match the color of most shirt waists and collars, and is soluble in water and rendered adhesive under the application of moisture and heat so that the support may be applied to a collar during the 60 ironing operation and removed therefrom when the collar is immersed in water for the purpose of laundering the same.

Having thus described the invention, what 65 is claimed as new is:

An adhesive compound for collar supports, the same consisting of glue, sixteen ounces, wax, eight ounces, and glycerin, three ounces, sufficient water being added to give the compound the proper consistency. 70

In testimony whereof I affix my signature in presence of two witnesses.

HENRY J. TILL. [L. s.]

Witnesses:

E. J. TROWBRIDGE,  
R. J. BROXHOLME.